

[54] **METHOD OF OBTAINING DUCTILE BERYLLIUM**

[75] Inventors: **William Taylor**, Wyomissing; **William O. Frauson**, Conyngham; **Stanley Chinowsky**, Reading, all of Pa.

[73] Assignee: **Kawecki Berylco Industries, Inc.**, New York, N.Y.

[22] Filed: **Mar. 25, 1971**

[21] Appl. No.: **127,972**

[52] U.S. Cl. .... **148/11.5 F**, 75/150, 148/13

[51] Int. Cl. .... **C22f 1/18**

[58] Field of Search .... 75/150; 148/11.5 R, 11.5 F, 148/13 R, 32

[56] **References Cited**

UNITED STATES PATENTS

3,065,117 11/1962 Brown et al. .... 148/13

|           |         |                    |          |
|-----------|---------|--------------------|----------|
| 3,349,597 | 10/1967 | Gross, Jr. ....    | 75/150 X |
| 3,333,994 | 8/1967  | Mallen et al. .... | 148/13   |
| 2,872,363 | 2/1959  | Macherey ....      | 148/11.5 |

OTHER PUBLICATIONS

Beryllium Ingot Sheet, Technical Bulletin No. 2210, The Beryllium Corporation, Reading, Pa., 1965.

Primary Examiner—Richard O. Dean

Attorney, Agent, or Firm—Pennie, Edmonds, Morton, Taylor & Adams

[57] **ABSTRACT**

A critical relationship is described between the rate of cooling of beryllium from a stress-relieving or forming temperature and the indigenous iron-to-aluminum impurity ratio in mechanically worked beryllium, with resulting improvement in its ultimate ductility.

**2 Claims, 1 Drawing Figure**



PATENTED FEB 12 1974

3,791,878



INVENTORS  
WILLIAM TAYLOR  
WILLIAM O. FRAUSON  
STANLEY CHINOWSKY  
BY

*Pennie, Edwards, Norton, Taylor & Adams*  
ATTORNEYS

## METHOD OF OBTAINING DUCTILE BERYLLIUM

This invention relates to beryllium metal and, more particularly, to a method of producing mechanically worked beryllium in ductile form.

Beryllium can be mechanically worked, as by rolling, extrusion or forming. When these operations introduce internal stresses in the beryllium product the stress must be relieved by an annealing-type heat treatment. A forming or annealing temperature of at least about 1,300°F., and preferably of about 1,370°F., is used and heating at temperature is carried out generally for from 20 minutes to as much as 2 hours. Following this heating, the beryllium is allowed to cool slowly as in the annealing of other metals, and slow cooling is generally effected by allowing the metal product to remain in the heat-treatment furnace while the furnace is allowed to cool to close to ambient temperature, a cooling rate that generally is of the order to 50°F. per hour. In the case of worked but previously ductile beryllium, it has been found that this type of annealing treatment frequently causes embrittlement of the beryllium to the extent that it exhibits virtually no elongation at its breaking point under tensile testing in a direction transverse to the working direction.

We have now discovered that the transverse embrittlement of mechanically worked but previously ductile consolidated beryllium occurs during forming or stress relieving by heat treatment when the ratio of iron to aluminum, both indigenous impurities in beryllium, exceeds a certain value with respect to the total amount of these two impurities, and further that embrittlement of such beryllium can be avoided by relatively fast cooling of the heat-annealed beryllium through a critical portion of its cooling temperature range. That is, we have developed an improvement in the forming or stress relieving by heat treatment of mechanically worked beryllium having a total indigenous iron plus aluminum purity content not substantially in excess of 0.3 percent by weight present in a ratio of iron to aluminum greater than that represented by the line AB in the FIGURE of the drawing. In this stress relieving, the worked beryllium is heated to a temperature of at least about 1,300°F. and we have found that the pre-stress relief transverse ductility of the beryllium is at least fully restored by cooling the heated beryllium at least as rapidly as can be effected by cooling in the ambient air through the cooling range of about 800°F. to about 500°F.

These and other novel features of the invention will be more readily understood from the following description taken in conjunction with the accompanying drawing in which

The FIGURE is a graph showing a line of critical indigenous iron-to-aluminum impurity ratios for varying

amounts of these impurities normally present in ductile consolidated beryllium.

Beryllium metal of commercial grade generally contains between about 700 to 2,000 ppm of iron and between about 100 and 1,400 ppm of aluminum as indigenous impurities. The ratio of iron to aluminum may vary widely in the grade unless special procedures are used to control the ratio. In exploring the effects of various impurities on the ductility of stress-relieved specimens of beryllium which had been mechanically worked by extrusion, we discovered that the transverse ductility of the stress-relieved specimen was virtually destroyed when the iron:aluminum ratio for various amounts of iron and aluminum were higher than, i.e., to the right and below, the values represented by the line AB in the FIGURE. Conversely, the transverse ductility remained unchanged during stress-relieving when the iron:aluminum ratio for various amounts of iron and aluminum were lower than, i.e., to the left and above, the values represented by the line AB in the FIGURE.

In further investigation of the cause or factors that influenced destruction of transverse ductility in the aforementioned specimens during stress-relieving specimens having a higher iron:aluminum ratio than that represented by line AB in the FIGURE, we discovered that the embrittlement occurred during a specific portion of the cooling operation, to wit, during the period that the specimens were passed through the range of approximately 800°F. to approximately 500°F. as they were being furnace cooled at a conventional furnace-cooling rate of about 50°F. per hour by turning off the source of furnace heat. By diminishing the time that the specimens were permitted to remain at a temperature within this range, we found that the transverse ductility of the stress-relieved specimens could be retained and sometimes increased. To do this, we found that the specimens should be cooled through the range of 800°F. to 500°F. at a rate at least as fast as that obtained by removing the specimens from the furnace at about 800°F. and by allowing them to cool in the ambient atmospheric air, e.g., at a rate of at least about 1,000°F. per hour, so that the specimens had passed through the critical cooling temperature range in about 20 minutes. Still more rapid cooling is possible by directing an air blast against the specimens during this temperature interval. After the specimens had been cooled to at least 500°F., they could be continued to be cooled in air or they could be returned to a furnace at a temperature no higher than 500°F. and allowed to cool with the furnace at a conventional furnace-cooling rate.

The influence of cooling rate after stress-relieving on slabs of beryllium extruded from ductile consolidated beryllium of the type described hereinbefore is shown by the data in the following table:

TABLE I

| Fe ppm | Al ppm | Fe/Al Ratio | Stress-relieving Conditions | U.T.S. (ksi $\times 10^3$ ) | Transverse 0.2% Y.S. (ksi $\times 10^3$ ) | Transverse Elongation % |
|--------|--------|-------------|-----------------------------|-----------------------------|-------------------------------------------|-------------------------|
| 1860   | 590    | 3.1         | None                        | 42.8                        | 34.9                                      | 0.8                     |
|        |        |             | 2 hr. 1370°F, S.C.*         | 42.2                        | nil                                       | nil                     |
|        |        |             | 2 hr. 1370°F, F.C.**        | 45.9                        | 41.2                                      | 0.5                     |
| 1570   | 150    | 10.5        | None                        | 52.7                        | 45.1                                      | 0.3                     |
|        |        |             | 2 hr. 1370°F, S.C.          | 49.0                        | nil                                       | nil                     |
|        |        |             | 2 hr. 1370°F, F.C.          | 56.3                        | 50.6                                      | 1.2                     |
| 1390   | 170    | 8.2         | None                        | 48.8                        | 42.0                                      | 0.5                     |
|        |        |             | 2 hr. 1370°F, S.C.          | 44.6                        | nil                                       | nil                     |
|        |        |             | 2 hr. 1370°F, F.C.          | 48.1                        | 40.9                                      | 0.8                     |

TABLE I - Continued

| Fe ppm | Al ppm | Fe/Al Ratio | Stress-relieving Conditions | U.T.S. (ksi $\times 10^3$ ) | Transverse 0.2%<br>% Y.S. (ksi $\times 10^3$ ) | Transverse<br>Elongation % |
|--------|--------|-------------|-----------------------------|-----------------------------|------------------------------------------------|----------------------------|
| 1380   | 180    | 7.7         | None                        | 56.5                        | 47.0                                           | 0.8                        |
|        |        |             | 2 hr. 1370°F, S.C.          | 59.9                        | nil                                            | nil                        |
|        |        |             | 2 hr. 1370°F, F.C.          | 57.8                        | 50.7                                           | 1.2                        |
| 1240   | 400    | 3.1         | None                        | 50.9                        | 45.5                                           | 1.0                        |
|        |        |             | 2 hr. 1370°F, S.C.          | 44.2                        | nil                                            | nil                        |
|        |        |             | 17 hr. 1370°F, F.C.         | 50.5                        | 45.1                                           | 1.0                        |

\*Slow cool in furnace at 50°F. per hour

\*\*Fast cool in ambient atmosphere

The following table presents data that shows that slow cooling does not have any significant detrimental effect on the transverse ductility of similar slabs of extruded beryllium where the only difference is an iron-aluminum ratio lower than that represented by the line AB in the FIGURE:

15 in excess of 0.3% by weight percent in a ratio of iron to aluminum greater than that represented by the line AB in the FIGURE of the drawing and the beryllium having been treated to a temperature above about 800°F., the improvement which comprises cooling the heated beryllium at least as rapidly as can be effected

TABLE II

| Fe ppm | Al ppm | Fe/Al Ratio | Stress-relieving Conditions | U.T.S.,<br>(ksi $\times 10^3$ ) | (ksi $\times 10^3$ ) | Elongation % |
|--------|--------|-------------|-----------------------------|---------------------------------|----------------------|--------------|
| 690    | 420    | 1.65        | None                        | 42.6                            | 35.6                 | 0.9          |
|        |        |             | 2 hr. 1370°F, S.C.*         | 41.1                            | 33.7                 | 0.9          |
| 1300   | 820    | 1.58        | None                        | 49.8                            | 43.7                 | 0.6          |
|        |        |             | 2 hr. 1370°F, S.C.*         | 47.0                            | 42.8                 | 0.5          |
| 1280   | 1020   | 1.25        | None                        | 53.3                            | 43.7                 | 0.7          |
|        |        |             | 2 hr. 1370°F, S.C.*         | 50.1                            | 40.2                 | 0.7          |
| 1580   | 1370   | 1.16        | None                        | 50.8                            | 43.1                 | 0.6          |
|        |        |             | 2 hr. 1370°F, S.C.*         | 47.1                            | 40.6                 | 0.4          |
| 700    | 1290   | 0.55        | None                        | 48.9                            | 40.8                 | 0.7          |
|        |        |             | 2 hr. 1370°F, S.C.*         | 48.0                            | 39.5                 | 0.8          |
| 1570   | 780    | 2.0         | None                        | 49.8                            | 43.5                 | 0.5          |
|        |        |             | 2 hr. 1370°F, S.C.*         | 47.9                            | 41.6                 | 0.5          |

\*Slow cool in furnace at 50°F. per hour

We claim:

1. In the cooling of mechanically worked beryllium which has been heated for the purpose of forming or stress-relieving, the beryllium having a total indigenous iron plus aluminum impurity content not substantially

40 by cooling in the ambient atmospheric air through the cooling range of about 800°F. to about 500°F.

2. The method according to claim 1 in which the heated beryllium is cooled at a rate of at least about 1,000°F. per hour through the cooling range of about 800°F. to about 500°F.